

# United States Patent [19]

Sakamoto et al.

[11] 3,769,017

[45] Oct. 30, 1973

[54] PHOTOSENSITIVE SILVER HALIDE ELEMENT CONTAINING A THIOSUGAR ANTIFOGGANT

[75] Inventors: Kenro Sakamoto; Isamu Fushiki; Shinji Arai; Fumio Shimizu; Yoshimi Kuwabara; Tomio Nakajima, all of Tokyo; Sadao Sugita, Hanno; Hiroyuki Inokuma, Kanagawa; Setsuko Tejima, Nagoya, all of Japan

[73] Assignee: Konishiroku Photo Industry Co., Ltd., Tokyo, Japan

[22] Filed: Mar. 29, 1972

[21] Appl. No.: 239,343

[52] U.S. Cl. .... 96/76 R, 96/109

[51] Int. Cl. .... G03c 1/34, G03c 1/76

[58] Field of Search..... 96/109, 107, 76 R

[56]

## References Cited

### UNITED STATES PATENTS

|           |         |                  |        |
|-----------|---------|------------------|--------|
| 3,635,717 | 1/1972  | Ohi et al. ....  | 96/108 |
| 3,297,446 | 1/1967  | Dunn ....        | 96/107 |
| 3,475,175 | 10/1969 | King et al. .... | 96/109 |

Primary Examiner—Norman G. Torchin

Assistant Examiner—Won H. Louie, Jr.

Attorney—Jordan B. Bierman et al.

[57]

## ABSTRACT

A photographic element comprising a support having thereon one or more layers at least one of which is a light-sensitive silver halide emulsion layer, said element contains at least one of certain thiosugars in an amount effective to inhibit fog.

9 Claims, No Drawings

# PHOTOSENSITIVE SILVER HALIDE ELEMENT CONTAINING A THIOSUGAR ANTIFOGGANT

This invention relates to light-sensitive silver halide photographic materials containing certain thiosugars.

When developed at relatively high temperatures, light-sensitive silver halide photographic materials tend to suffer from fogging, in general. This phenomenon is considered ascribable to the fact that the activation energy required for the development of fog is greater than that required for the development of photographic image. Accordingly, the development of photographic materials at elevated temperatures is not so desirable. As the quick processing of light-sensitive photographic materials have been demanded recently, however, the time required for development is intended to be shortened. Owing to such quick development, it has been found that many substances, which have been effectively used as antifoggants hitherto, have various drawbacks in practice. For example, there are encountered the cases where a certain compound, when used in an amount within a range capable of sufficiently inhibiting the formation of fog at the time of high temperature development, brings about such drawbacks as to greatly decrease the speed, or to degrade the developability, of the resulting photographic material, or to cause, in the case of a color photographic material, insufficient bleaching of metallic silver after color development of the photographic material.

An object of the present invention is to provide light-sensitive silver halide photographic materials suitable for quick development at elevated temperatures.

Another object of the invention is to provide light-sensitive silver halide photographic materials which scarcely form fog even when the development time is prolonged.

A further object of the invention is to provide light-sensitive silver halide photographic materials which are less in variation of photographic properties even when stored for a long period of time.

Other objects and advantages of the invention will become apparent from the description made hereinbelow.

In accordance with the present invention, there are provided light-sensitive silver halide photographic materials containing thiosugars of the general formula,



wherein  $R_1$  is a hydrogen atom, an alkyl group, or a group of the formula



(where X is a halogen atom).



(where Y and Z are individually an alkyl, aryl or aralkyl group); R<sub>2</sub> is a hydrogen atom or a group of the for-

mula  $-\text{CH}_2-\text{O}-\text{R}_3$  (where  $\text{R}_3$  is an acyl group). Further, all the stereoisomers with respect to  $\text{C}_{(1)}$  to  $\text{C}_{(5)}$  are included by the thiosugars.

When one or more of the above-mentioned thiosugars are incorporated into at least one of the layers (e.g. emulsion layer, sub layer, protective layer, backing layer or the like) of a light-sensitive silver halide photographic material, said photographic material is successfully inhibited from formation of fog to make it possible to accomplish the above-mentioned objects of the present invention. That is, even when the said photographic material is subjected to high temperature treatment, not only the formation of fog and the formation of stains (stains formed by reaction of couplers contained in the photographic material with an oxidation product of the developer used for the development thereof) can effectively be inhibited, but also the tendency of forming said fog and stains can successfully be suppressed even when the development time is prolonged.

20 The thiosugars of the aforesaid general formula can be synthesized according to, for example, the process disclosed in Journal of the American Chemical Society, 70 2598 (1958). Typical examples of said thiosugars are as follows:

1. Triacetyl-L-arabinose isothiuronium bromide
  2. Triacetyl-D-xylose isothiuronium bromide
  3. 1-Methylthio-D-xylose triacetate
  4. Amyl triacetyl-L-arabinose xanthate
  5. 1-Mercapto-D-xylose triacetate
  6. Benzyl triacetyl-L-arabinose xanthate
  7. Ethyl triacetyl-D-xylose xanthate
  8. Amyl tetraacetyl-D-mannose xanthate
  9. Butyl tetraacetyl-D-glucose xanthate
  10. 1-Mercapto-D-glucose tetraacetate
  11. 1-Acetylthio-D-mannose tetraacetate
  12. Tetraacetyl-D-glucose isothiuronium bromide
  13. Benzyl triacetyl-D-ribose xanthate
  14. m-Tolyl tetraacetyl-D-glucose xanthate
  15. Ethyl triacetyl-D-ribose xanthate
  16. 1-Methylthio-D-glucose tetraacetate
  17. 1-Acetylthio-D-ribose triacetate
  18. 1-Mercapto-D-mannose tetraacetate
  19. Phenyl tetracetyl-D-mannose xanthate
  20. 1-Laurylthio-D-mannose tetraacetate
  21. 1-Benzoylthio-D-glucose tetraacetate

Typical procedures for synthesizing the above-mentioned thiosugars are set forth below with reference to synthesis examples.

### SYNTHESIS EXAMPLE 1

### Synthesis of n-butyl tetraacetyl-D-glucose xanthate [the exemplified compound (9)]:

1. Into a mixture comprising 12 g. of D-glucose and 46.8 cc. of acetic anhydride were dropped several drops of concentrated sulfuric acid. After heating the mixture over a water bath for 2 hours, acetic acid was removed by distillation under reduced pressure. The residue was poured into ice water, and the resulting liquid was stirred to deposit crystals. Subsequently, the crystals were recovered by filtration, washed with water and then dried to obtain D-pentaacetyl glucose, yield 20.4 g.

2. A mixture comprising 10 g. of the thus obtained D-pentaacetyl glucose, 10 cc. of a 30 percent hydrogen bromide-acetic acid solution and 5 cc. of acetic acid was stirred at room temperature for 2 hours in a means shielded from moisture, and then gradually dropped

into ice water, which was kept with vigorous stirring, to deposit crystals. The crystals were quickly collected by filtration and immediately transferred into ether. The resulting ether solution was washed with a dilute aqueous sodium bicarbonate solution and dried over sodium sulfate, and then the ether was removed by distillation under reduced pressure. The residue was extracted with petroleum ether, and the extract was cooled to deposit crystals, which were then recovered by filtration and dried under reduced pressure to obtain D-acetobromoglucose in the form of white crystalline needles, m.p. 88°-89°C., yield 4 g.

3. 2 Grams of the thus obtained D-acetobromoglucose was added to a suspension of 0.9 g. of potassium n-butyl xanthate in 10 cc. of ethanol, and the suspension was refluxed over a water bath for 10 minutes. After cooling, the liquid reaction mixture was poured into 60 cc. of water, and then cooled to deposit crystals. Subsequently, the crystals were recovered by filtration, washed with water, dried under reduced pressure and then recrystallized from a small amount of ethanol to obtain butyl D-tetraacetyl glucose xanthate in the form of pale yellowish white crystals, m.p. 115°-116°C., yield 1.7 g.

Elementary analysis for  $C_{19}H_{28}O_{10}S_2$ :

Found (%) C: 47.51 H: 6.01 S: 12.68

Calculated (%) C: 47.49 H: 5.87 S: 13.35

#### Synthesis Example 2

Synthesis of tetraacetyl-D-glucose isothiuronium bromide [the exemplified compound (12)]:

A mixture comprising 2 g. of D-acetobromo-glucose, 0.4 g. of thiourea and 4 cc. of acetone was refluxed over a water bath for 15 minutes, and then cooled to deposit crystals. The crystals were dissolved in 150 cc. of acetone, and the resulting solution was subjected to filtration to remove insoluble matters. Thereafter, the filtrate was concentrated under reduced pressure to one-third the original volume, and then cooled to deposit crystals. Subsequently, the crystals were recovered by filtration and dried under reduced pressure to obtain tetraacetyl-D-glucose isothiuronium bromide in the form of white crystals, m.p. 204°C., yield 0.6 g.

Elementary analysis for  $C_{15}H_{23}N_2O_9BrS$

Found (%) C: 36.39 H: 4.94 N: 6.01

Calculated (%) C: 36.97 H: 4.76 N: 5.75

Br: 16.40 S: 6.58

The thiosugar used in the present invention may be incorporated into any of the layers of a light-sensitive photographic material, and is most preferably added to a photographic emulsion which has completed the second ripening. Alternatively, however, the thiosugar may be added before or during the second ripening to control the progress of the ripening, or may have previously been incorporated into gelatin or the like starting material for preparation of the emulsion. Furthermore, the thiosugar may be applied to a light-sensitive color photographic material of the so-called protect type in which the thiosugar is made present together with water-insoluble or scarcely water-soluble couplers and is dissolved in a water-immiscible high boiling solvent and the resulting solution is dispersed in the emulsion. The amount of the thiosugar to be added varies depending on the kind of the emulsion used, the kind of the compound and the desired fog-inhibiting conditions. Generally, however, the thiosugar is used in an amount of 10 mg. to 2 g. per mole of silver halide and may be

added in the form of a solution in a suitable organic solvent such as, for example, methanol, ethanol, acetone or ethyl acetate. In case the thiosugar is desired to be incorporated into an auxiliary layer other than the emulsion layer, it is preferable that the amount of the thiosugar added is controlled so that the total amount thereof per unit area of the resulting photographic material becomes an amount corresponding to the above-mentioned amount. If necessary, however, the amount may be increased to a suitable extent.

The aforesaid objects of the present invention can be accomplished more successfully by incorporating into a light-sensitive photographic material the thiosugar in combination with a high molecular compound such as 15 poly-N-pyrrolidone or a copolymer of N-vinylpyrrolidone with another ethylenically polymerizable compound. Typical examples of the above-mentioned high molecular compound are as follows:

|                                                                                            | Monomer ratio |
|--------------------------------------------------------------------------------------------|---------------|
| 22. Poly-N-vinyl-2-pyrrolidone                                                             | 42:58         |
| 23. N-Vinylpyrrolidone/imidazolinoacrylic amide copolymer                                  | 42:58         |
| 24. N-Vinylpyrrolidone/morpholinoacrylic amide copolymer                                   | 42:58         |
| 25. N-Vinylpyrrolidone/piperidinoacrylic amide copolymer                                   | 42:58         |
| 26. N-Vinylpyrrolidone/2-methylimidazolinoacrylic amide copolymer                          | 42:58         |
| 27. N-Vinylpyrrolidone/acrylic diethylamide copolymer                                      | 42:58         |
| 28. N-Vinylpyrrolidone/sodium acrylate copolymer                                           | 75:25         |
| 29. N-Vinylpyrrolidone/methyl acrylate copolymer                                           | 42:58         |
| 30. N-Vinylpyrrolidone/acrylic amide copolymer                                             | 75:25         |
| 31. N-Vinylpyrrolidone/ethyl acrylate copolymer                                            | 70:30         |
| 32. N-Vinylpyrrolidone/acrylic amide/ammonium maleamate copolymer                          | 40:40:20      |
| 33. N-Vinylpyrrolidone/acrylic amide/maleic anhydride copolymer                            | 40:40:20      |
| 34. N-Vinylpyrrolidone/acrylic amide/2-methylimidazolone copolymer                         | 60:20:20      |
| 35. N-Vinylpyrrolidone/acrylic amide/sodium 2-methylimidazole-3-hydro-propionate copolymer | 60:20:20      |
| 36. N-Vinylpyrrolidone/imidazolinomaleamic acid imidazole salt copolymer                   | 60:40         |
| 37. N-Vinylpyrrolidone/2-methylimidazolino-maleamic acid 2-methylimidazole salt copolymer  | 60:40         |
| 38. N-Vinylpyrrolidone/2-methylimidazole copolymer                                         | 60:40         |
| 39. N-Vinylpyrrolidone/morpholinomethacrylic acid/methyl methacrylate copolymer            | 20:20:60      |
| 40. N-Vinylpyrrolidone/4-vinylpyridino-N-methyl iodide copolymer                           | 42:58         |
| 41. N-Vinylpyrrolidone/piperidinomaleamic acid piperidine salt copolymer                   | 60:40         |
| 42. N-Vinylpyrrolidone/maleic acid thiourea half ammonium salt copolymer                   | 60:40         |
| 43. N-Vinylpyrrolidone/styrene copolymer                                                   | 70:30         |
| 44. N-Vinylpyrrolidone/piperidino methacrylate/methyl methacrylate copolymer               | 20:20:60      |
| 45. N-Vinylpyrrolidone/methacrylic amide/methyl methacrylate copolymer                     | 20:20:60      |
| 46. N-Vinylpyrrolidone/vinyl acetate copolymer                                             | 70:30         |

When any one of the above-mentioned high molecular compounds is incorporated in combination with at least one of the aforesaid thiosugars into a light-sensitive silver halide photographic material, a more excellent antifogging effect can be attained at the time of high temperature processing than in the case where the thiosugar is used alone.

The above-mentioned high molecular compound is dissolved in water or an alkali solution or in such an organic solvent as methanol, ethanol, acetone, ethyl acetate, dioxane or dimethylformamide, and the resulting

solution is added to a coating liquid for forming an emulsion layer or an auxiliary layer. The amount of the compound to be used in the above case varies depending on various factors such as the kinds of the compound, the thiosugar used and the layer to which the compound is added, and the like, but is ordinarily within the range from 0.2 to 100 g. per mole of silver halide. In the above case, the amount of the thiosugar to be added is preferably within the aforesaid range. In case the high molecular compound is desired to be incorporated into an internal color photographic material containing an oil-soluble coupler, i.e. a so-called protect type coupler, the compound may be dissolved in a solvent for said coupler or added to a dispersion of said coupler, and then incorporated into, for example, an emulsion layer.

The light-sensitive silver halide photographic materials according to the present invention include photographic materials of various types such as, for example, color photographic materials, black-and-white photographic materials, roentgen photographic materials, other radiation-sensitive photographic materials, light-sensitive printing materials and diffusion transfer type printing materials.

The silver halides used in the present invention include silver chloride, silver bromide, silver chlorobromide, silver iodobromide, etc., and the emulsions containing said silver halides may be optically sensitized by use of various sensitizing dyes such as cyanine dyes, merocyanine dyes or styryl dyes, or may be chemically sensitized by use of such chemical sensitizers as sulfur-containing compounds, noble metal salts, polyalkylene oxide derivatives or reducing compounds. Further, as the hydrophilic protective colloids employed as binders in the above case, or as other layer-forming components, gelatin is used, in general, but other known hydrophilic protective colloids, e.g. polyvinyl alcohols and the like, may also be used.

The light-sensitive photographic materials according to the present invention may contain various photographic additives, e.g. coating aids such as lauryl or oleyl monoethers of saponin or polyethylene glycol, or sulfonated or alkylated polyethylene glycol ether salts; stabilizers or inhibitors such as triazaindolizine type compounds or mercaptotetrazole type compounds; hardeners such as mucobromic acid and the like; halogen-substituted fatty acids, or formaldehyde; couplers such as yellow couplers having benzoyl acetanilide groups or the like, magenta couplers having pyrazolone nuclei, indazolone nuclei or cyanoacetyl groups, and cyan couplers having phenol or naphthol nuclei (these couplers may have in the active methylene or methine positions such substituents as halogen atoms or allylazo, allyloxy or allylthio groups capable of being released by color development reaction, and may have in the molecules such non-diffusing groups as long chain alkyl groups or alkylphenoxy groups or such water-soluble groups as sulfonic acid groups or carboxyl groups); and plasticizers such as glycerin and the like. Even when these photographic additives are made present together with the thiosugars, they have no detrimental interactions on the photographic properties of the photographic materials.

In incorporating the aforesaid couplers into the light-sensitive photographic materials, there may be adopted the procedures mentioned below. That is, the protect type couplers are dissolved in such high boiling organic

solvent as dibutyl phthalate or in such solvent as chloroform, acetone or dimethylformamide and then dispersed in the emulsions, while the couplers having water-soluble groups are dissolved in an alkali solution and then incorporated into the emulsions. On the other hand, some of the couplers are incorporated into color developers and are used as the so-called external couplers.

The light-sensitive color photographic materials are composed of, in general, yellow layer, yellow filter layer, magenta layer, inter layer, cyan layer, antihalation layer and support in this order from the uppermost layer, though the order of the yellow, magenta and cyan layers may sometimes be varied. In this case, each of the color-forming layers such as the yellow layer and the like may be composed of one or two layers.

Supports for the light-sensitive photographic materials according to the present invention are suitably selected in consideration of the application purposes of the photographic materials, and include papers, laminated papers, and natural and synthetic high molecular films of the cellulose acetate and polyester types. If necessary, these supports may be subjected to subbing or the like hydrophilization to make the coating of hydrophilic protective colloid easy and to make the adhesion thereof strong.

The development of the present light-sensitive silver halide photographic materials as mentioned above is carried out, in general, in the manner mentioned below. That is, the black-and-white photographic materials are ordinarily developed with a developer containing such developing agent as Metol, hydroquinone or phenidone; the negative type color photographic materials are ordinarily developed with a developer containing a color developing agent of the p-phenylenediamine type; and the positive type color photographic materials are ordinarily developed in such a manner that the photographic materials are initially subjected to black-and-white development and then subjected to color development. In the above-mentioned development, the photographic materials of the present invention display satisfactory antifogging effects not only at normal temperature of about 20° to 25°C, but also at elevated temperatures adopted at the time of quick processing. Moreover, even when the processing time is prolonged, the photographic materials are successfully inhibited from formation of color fog, are less in desensitization, and have excellent photographic properties.

The present invention is illustrated in detail below with reference to examples, but the examples are merely illustrative and do not limit the scope of the invention.

#### EXAMPLE 1

A high speed roentgen silver iodobromide emulsion containing 2 mole percent of silver iodide was subjected to second ripening, and incorporated with the following compounds:

|                                           |                   |
|-------------------------------------------|-------------------|
| 5-Methyl-7-hydroxy-1,3,4-triazaindolizine | 2.0 g/Ag × 1 mole |
| 3% Saponin                                | 30 ml/Ag × 1 mole |
| Mucochloric acid                          | 3 mg/g gelatin.   |

Subsequently, the emulsion was equally divided into four emulsions, and one emulsion was left as it was and

the other three emulsions were individually incorporated with such compounds as shown in Table 1. Thereafter, the four emulsions were individually coated on a polyester support and then dried to prepare light-sensitive films. These films were exposed to a definite light through an optical wedge, developed at 38°C. for 30, 45 and 60 seconds with a strongly alkaline roentgen film developer containing 1-phenyl-3-pyrazolidone and hydroquinone as developing agents, and then measured in speed and fog. The results obtained were as set forth in Table 1.

5% Sodium dodecylbenzenesulfonate — 100 ml.  
6. 3% Saponin — 60 ml/Ag  $\times$  1 mole

The thus obtained coating liquid was coated on a cellulose triacetate support to a dry film thickness of 3.5  $\mu$  and then dried to prepare a photographic film. This film was exposed to a definite light through an optical wedge and then subjected to the following processings: Processings:

10 1. Prehardening 40°C. 60 sec.  
2. Neutralization " 20 "

TABLE 1

| Kind of compound                | Amount of compound (g/Ag $\times$ 1 mole) | 30 sec.        |      | 45 sec.        |      | 60 sec.        |      |
|---------------------------------|-------------------------------------------|----------------|------|----------------|------|----------------|------|
|                                 |                                           | Relative speed | Fog  | Relative speed | Fog  | Relative speed | Fog  |
| None .....                      | .....                                     | 100            | 0.50 | 100            | 0.76 | 100            | 0.98 |
| Exemplified compound (26) ..... | 5.5                                       | 100            | .46  | 100            | .65  | 108            | .75  |
| Exemplified compound (17) ..... | 1.5                                       | 100            | .13  | 110            | .25  | 115            | .32  |
| Exemplified compound (26) ..... | 5.5                                       | 100            | .13  | 120            | .18  | 138            | .26  |
| Exemplified compound (17) ..... | 1.5                                       | 100            | .13  | 120            | .18  | 138            | .26  |

(In the above table, the relative speed is a value measured by assuming as 100 the speed of the blank sample at each development time.)

From Table 1, it is understood that even when used alone, the thiosugar [the exemplified compound (17)] can successfully inhibit the photographic material from formation of fog without giving any detrimental influence to the speed thereof as compared with the case of the photographic material incorporated with no such compound, and that when the said compound is used in combination with the high molecular compound [the exemplified compound (26)], the degree of increase in fog of the photographic material is markedly low even when the development time is prolonged, and the time permissible for the high temperature development thereof is broadened to a great extent.

## EXAMPLE 2

A high speed silver iodobromide emulsion containing 5 mole percent of silver iodide was subjected to second ripening and incorporated with the below-mentioned photographic additives (1) to (6) in this order to obtain a green-sensitive coating liquid.

1. 3,3'-Diethyl-5,5'-diphenyl-9-ethyl-oxacarbocyanine bromide — 0.14 g/Ag  $\times$  1 mole.
2. 5-Methyl-7-hydroxy-1,3,4-triazaindolizine — 1.4 g/Ag  $\times$  1 mole
3. 1-Phenyl-5-mercaptotetrazole — 0.05 g/Ag  $\times$  1 mole
4. Each of such combinations as shown in Table 2 of thiosugars and high molecular compounds used in the present invention.
5. A coupler dispersion prepared by subjecting to a high speed rotary mixer a mixture of the following composition (per Ag  $\times$  1 mole):  
1-(2',4',6'-Trichlorophenyl)-3-[3''-(2'',4''-di-tert-aminophenoxy acetamide)-benzamide]-5-pyrazolone — 54 g.  
1-(2',4',6'-Trichlorophenyl)-3-[3''-(2'',4''-di-tert-aminophenoxy acetamide)-benzamide]-4-(4''-methoxyphenylazo)-5-pyrazolone — 17 g.  
Tricresyl phosphate — 55 g.  
Ethyl acetate — 85 g.  
3% Gelatin — 700 ml.

30 3. Color development " The time was varied as in Table 2.  
4. Stopping " 20 sec.  
5. Water-washing " 20 "  
6. Bleaching " 40 "  
7. Fixing " 60 "  
8. Water-washing " 40 "  
9. Stabilization " 20 "

Prescriptions:  
35 3. Color development " The time was varied as in Table 2.  
Prehardening bath (pH 4.9-5.0):

30 Sodium bisulfate 0.8 g.  
2,5-Dimethoxytetrahydrofuran 5.0 ml.  
Sodium sulfate 136.0 g.  
Formalin (35-40%) 30.0 ml.  
Potassium bromide 16.0 g.  
Water to make 1 liter

Neutralization bath (pH 5.1-5.2):

45 Acetic acid 1.5 ml.  
Sodium acetate 24.0 g.  
Potassium bromide 17.0 g.  
Sodium sulfate 25.0 g.  
Potassium metabisulfite 30.0 g.  
Water to make 1 liter

Color development bath (pH 10.65-10.70):

50 Benzyl alcohol 5 ml.  
Sodium sulfite 2 g.  
Sodium bromide 1.5 g.  
Sodium hydroxide 12 g.  
Borax 55 g.  
4-Amino-N-ethyl-N-( $\beta$ -metasulfonamidoethyl)-m-toluidine 3/2 H<sub>2</sub>SO<sub>4</sub>H<sub>2</sub>O 5 g.  
Water to make 1 liter

Stopping bath (pH 3.4-3.6):

60 Sodium acetate 5.3 g.  
Acetic acid 32.0 ml.  
Water to make 1 liter

Bleaching bath (pH 6.6-7.0):

65 Potassium ferricyanide 112.0 g.  
Potassium bromide 24.0 g.  
Disodium phosphate.7H<sub>2</sub>O 45.0 g.  
Monosodium phosphate 12.0 g.

Sodium thiocyanate 10.0 g.  
Water to make 1 liter

## Fixing bath:

Ammonium thiosulfate 120.0 g.  
Potassium metabisulfite 20.0 g.  
Water to make 1 liter

## Stabilization bath:

Formalin (35-40%) 3.0 ml.  
Kodak Stabilizer MX-707 (10%) 10.0 ml.  
Water to make 1 liter

The relative speed and fog of each film after the processings were as set forth in Table 2.

Ethyl acetate — 140 g.  
3% Gelatin — 700 ml.  
5% Sodium dodecylbenzenesulfonate — 100 ml.  
4. 3% Saponin — 95 ml/Ag  $\times$  1 mole  
5. 0.5% Mucochloric acid — 80 ml/Ag  $\times$  1 mole

The thus obtained coating liquid was coated on a cellulose triacetate support to a dry film thickness of 4  $\mu$  and then dried to prepare a photographic film. This film was exposed to a definite light through an optical wedge and then subjected to the following processings:

## Processings:

1. Prehardening 50°C. 35 sec.  
2. Neutralization " " 35 "  
3. First development " " The time was varied as in Table 3

TABLE 2

| Kind and amount (g/Ag $\times$ 1 mole) of thiosugar | Kind and amount (g/Ag $\times$ 1 mole) of high molecular compound | Developed for 1 min. |      | Developed for 2 min. |      | Developed for 3 min. |      |
|-----------------------------------------------------|-------------------------------------------------------------------|----------------------|------|----------------------|------|----------------------|------|
|                                                     |                                                                   | Relative speed       | Fog  | Relative speed       | Fog  | Relative speed       | Fog  |
| Exemplified compound (5) 0.7                        | Exemplified compound (22) 0.34 ....                               | 100                  | 0.20 | 100                  | 0.30 | 100                  | 0.52 |
| Exemplified compound (5) 0.7                        | Exemplified compound (22) 0.34 ....                               | 100                  | .18  | 100                  | .26  | 103                  | .40  |
| Exemplified compound (9) 0.7                        | Exemplified compound (22) 0.34 ....                               | 100                  | .13  | 101                  | .18  | 110                  | .24  |
| Exemplified compound (9) 0.7                        | Exemplified compound (22) 0.34 ....                               | 100                  | .06  | 105                  | .08  | 105                  | .08  |
| Exemplified compound (9) 0.7                        | Exemplified compound (22) 0.34 ....                               | 98                   | .12  | 100                  | .18  | 105                  | .22  |
| Exemplified compound (9) 0.7                        | Exemplified compound (22) 0.34 ....                               | 96                   | .07  | 102                  | .08  | 100                  | .10  |

As is clear from Table 2, it is understood that even when the thiosugar is used alone, considerable antifogging effect can be seen, but when the thiosugar is used in combination with poly-N-vinylpyrrolidone, markedly high antifogging effect can be attained without accompanying desensitization and, particularly, the variation in fog value due to the development time variation becomes smaller.

## EXAMPLE 3

A high speed silver iodobromide emulsion containing 3.5 mole percent of silver iodide was subjected to second ripening and incorporated with the below-mentioned photographic additives (1) to (5) in this order to obtain a red-sensitive emulsion.

1. 3,3'-Diethyl-5,5'-dichloro-9-ethyl-thiacarbocyanine iodide — 0.12 g/Ag  $\times$  1 mole

2. Each of such combinations as shown in Table 3 of thiosugars and high molecular compounds used in the present invention.

3. A coupler dispersion prepared by subjecting to a high rotary mixer a mixture of the following composition (per Ag  $\times$  1 mole):

1-Hydroxy-2-[ $\alpha$ -(2', 4'-di-tert-amylphenoxy)-n-(butyl)]naphthamide — 48 g.

Tricresyl phosphate — 20 g.

30 4. First stopping " 35 sec.  
5. Water-washing " 35 "  
6. Supplementary exposure " About 10 "  
7. Color development " 120 "  
8. Second stopping " 35 "  
9. Water-washing " 35 "  
10. Bleaching " 35 "  
11. Fixing " 35 "  
12. Water-washing " 60 "  
13. Stabilization " 35 "  
(The operations 5-13 may be effected under an ordinary room light.)

## Formulations

40 Same as in Example 2 except the first development bath. First development bath (pH 10.1-10.3):

|                                  |         |
|----------------------------------|---------|
| Sodium hexametaphosphate         | 2.0 g.  |
| Metol                            | 6.0 g.  |
| Sodium sulfite                   | 50.0 g. |
| Sodium carbonate                 | 30.0 g. |
| Hydroquinone                     | 6.0 g.  |
| Potassium bromide                | 2.0 g.  |
| Sodium thiocyanate               | 1.3 g.  |
| Sodium hydroxide                 | 2.0 g.  |
| Potassium iodide (0.1% solution) | 60 ml.  |
| Water to make                    | 1 liter |

The relative speed and maximum density (D-max) of each film after the processings were as set forth in Table 3.

TABLE 3

| Kind and amount (g/Ag $\times$ 1 mole) of thiosugar | Kind and amount (g/Ag $\times$ 1 mole) of high molecular compound | Developed for 45 sec. |       | Developed for 60 sec. |       | Developed for 75 sec. |       |
|-----------------------------------------------------|-------------------------------------------------------------------|-----------------------|-------|-----------------------|-------|-----------------------|-------|
|                                                     |                                                                   | Relative speed        | D-max | Relative speed        | D-max | Relative speed        | D-max |
| Exemplified compound (11) 2.0                       | Exemplified compound (30) 5.5 ....                                | 100                   | 2.32  | 100                   | 2.08  | 100                   | 1.76  |
| Exemplified compound (11) 2.0                       | Exemplified compound (30) 5.5 ....                                | 100                   | 2.32  | 99                    | 2.14  | 96                    | 2.00  |
| Exemplified compound (11) 2.0                       | Exemplified compound (30) 5.5 ....                                | 100                   | 2.30  | 100                   | 2.18  | 101                   | 2.10  |
| Exemplified compound (16) 1.5                       | Exemplified compound (37) 2.0 ....                                | 100                   | 2.30  | 98                    | 2.30  | 98                    | 2.26  |
| Exemplified compound (16) 1.5                       | Exemplified compound (37) 2.0 ....                                | 100                   | 2.32  | 100                   | 2.16  | 95                    | 2.06  |
| Exemplified compound (16) 1.5                       | Exemplified compound (37) 2.0 ....                                | 100                   | 2.29  | 98                    | 2.15  | 100                   | 2.10  |
| Exemplified compound (16) 1.5                       | Exemplified compound (37) 2.0 ....                                | 100                   | 2.31  | 97                    | 2.30  | 96                    | 2.28  |

As is clear from Table 3, it is understood that in color reversal treatment also, an antifogging effect in the first development is seen by use of the thiosugar, with the result that the D-max value is maintained as it is without any substantial decrease in relative speed. This effect can be more enhanced by using the thiosugar in combination with containing a high molecular compound, e.g. N-vinylpyrrolidone.

#### EXAMPLE 4

A light-sensitive color printing paper having a protective layer, a red-sensitive layer, an inter layer, a green-sensitive layer, an inter layer, a blue-sensitive layer and a support in this order from the upper-most layer was prepared by successively coating emulsions of the below-mentioned compositions on a baryta paper to form respective layers.

##### 1. Blue-sensitive layer

A silver chloroiodobromide emulsion containing 1.3 mole percent of silver iodide and 15 mole percent of silver bromide was subjected to second ripening and successively incorporated with such photographic additives as mentioned below.

$\alpha$ -[4-( $\beta$ -Carboxy- $\beta$ -octadecyl propionylamide)-benzoyl]-3-carboxy-6-methoxyacetanilide — 100 g.

3% Saponin — 80 ml.

0.5% Mucochloric acid — 110 ml.

Subsequently, the emulsion was coated on a baryta paper to a dry film thickness of 4.0  $\mu$  and then dried to form a blue-sensitive layer.

##### 2. Inter layer

An emulsion of the composition shown below was coated on the above-mentioned blue-sensitive layer to a dry film thickness of 1  $\mu$  and then dried to form an inter layer.

2% Gelatin — 960 ml.

3% Saponin — 30 ml.

0.5% Mucochloric acid — 35 ml.

##### 3. Green-sensitive layer

A silver chlorobromide emulsion containing 15 mole percent of silver bromide was successively incorporated with such photographic additives as mentioned below.

3,3'-Diethyl-5,5'-diphenyl-9-ethyl-oxacarbocyanine bromide — 0.28 g.

1-Phenyl-3-( $\beta$ -carboxy- $\beta$ -octadecyl-propionylamide)-5-pyrazolone — 80 g.

3% Saponin — 80 ml.

0.5% Mucochloric acid — 110 ml.

Subsequently, the emulsion was coated on the above-mentioned inter layer to a dry film thickness of 3.5  $\mu$  and then dried to form a green-sensitive layer.

##### 4. Inter layer

An emulsion of the same composition as in the case of the aforesaid inter layer (2) was coated on the above-mentioned green-sensitive layer to a dry film thickness of 1  $\mu$  and then dried to form an inter layer.

##### 5. Red-sensitive layer

A silver chlorobromide emulsion containing 15 mole percent of silver bromide was subjected to second ripening and successively incorporated with such photographic additives as mentioned below.

3,3'-Diethyl-5,6,5',6'-dibenzo-9-ethyl-thiacarbocyanine bromide — 0.25 g.

N-[3-( $\beta$ -Carboxyl- $\beta$ -octadecyl propionylamide) propyl]-1-hydroxy-2-naphthamide — 90 g.

3% Saponin — 80 ml.

0.5% Mucochloric acid — 110 ml.

5 Subsequently, the emulsion was coated on the above-mentioned inter layer to a dry film thickness of 3.5  $\mu$  and then dried to form a red-sensitive layer.

##### 6. Protective layer:

An emulsion of the same composition as in the case 10 of the aforesaid inter layer (2) was coated on the above-mentioned red-sensitive layer to a dry film thickness of 1  $\mu$  and then dried to form a protective layer.

The light-sensitive color printing paper prepared in the above manner was used as a control sample.

15 On the other hand, a sample was prepared in the same manner as above, except that a combination of 0.85 g./Ag  $\times$  1 mole of the exemplified compound (7) and 2.3 g./Ag  $\times$  1 mole of the exemplified compound (22) (PVPK-20 Powder, manufactured and sold by

20 General Aniline and Film Corporation) was incorporated into each of the blue-sensitive, green-sensitive and red-sensitive emulsions.

These samples were individually subjected to the following processings:

##### 25 Processings:

|                       |       |                                                      |
|-----------------------|-------|------------------------------------------------------|
| 1. Color development  | 30°C. | The development time was varied as shown in Table 4. |
| 2. Stop-fix-hardening | "     | 30 sec.                                              |
| 3. Water-washing      | "     | 30 "                                                 |
| 4. Bleach-fixing      | "     | 2 min.                                               |
| 5. Water-washing      | "     | 3 "                                                  |

##### Formulations:

###### Color development bath (pH 10.8-11.0):

|                                                                    |              |
|--------------------------------------------------------------------|--------------|
| Sodium hexametaphosphate                                           | 2.0 g.       |
| Hydroxylamine sulfate                                              | 4.0 g.       |
| Sodium sulfite                                                     | 4.0 g.       |
| 40 Potassium carbonate                                             | 60.0 g.      |
| Potassium bromide                                                  | 0.5 g.       |
| Sodium hydroxide                                                   | 6.0 - 8.0 g. |
| 4-Amino-N-ethyl-N-( $\beta$ -methane-sulfonamidoethyl)-m-toluidine |              |
| 3/2 H <sub>2</sub> SO <sub>4</sub> ·H <sub>2</sub> O               | 8.0 g.       |
| Water to make                                                      | 1 liter      |

###### 45 Stop-fix-hardening bath (pH 4.3 $\pm$ 0.1):

|                      |          |
|----------------------|----------|
| Ammonium thiosulfate | 100.0 g. |
| Sodium sulfite       | 20.0 g.  |
| Acetic acid (100%)   | 30.0 ml. |
| 50 Potassium alum    | 30.0 g.  |
| Sodium acetate       | 30.0 g.  |
| Water to make        | 1 liter  |

###### 55 Fix-bleaching bath (pH 6.9 $\pm$ 0.1):

|                                                 |          |
|-------------------------------------------------|----------|
| Ethylenediamine-tetraacetic acid NaFe           | 50.0 g.  |
| Ethylenediaminetetraacetic acid Na <sub>2</sub> | 5.0 g.   |
| Sodium carbonate                                | 3.0 g.   |
| 60 Ammonium thiosulfate                         | 120.0 g. |
| Sodium thiocyanate                              | 10.0 g.  |
| Sodium sulfite                                  | 10.0 g.  |
| Potassium iodide                                | 1.0 g.   |
| Water to make                                   | 1 liter  |

65 The variation in fog stability of each sample due to the variation of development time was as set forth in Table 4.

TABLE 4

| Sample                               | Developed for 3 min. |                |                | Developed for 4 min. |                |                | Developed for 5 min. |                |                |
|--------------------------------------|----------------------|----------------|----------------|----------------------|----------------|----------------|----------------------|----------------|----------------|
|                                      | D <sub>B</sub>       | D <sub>G</sub> | D <sub>R</sub> | D <sub>B</sub>       | D <sub>G</sub> | D <sub>R</sub> | D <sub>B</sub>       | D <sub>G</sub> | D <sub>R</sub> |
| Control sample.....                  | 0.02                 | 0.03           | 0.02           | 0.10                 | 0.09           | 0.13           | 0.22                 | 0.18           | 0.25           |
| Sample of the present invention..... | .02                  | .02            | .03            | .03                  | .04            | .04            | .05                  | .05            | .07            |

(In the table; D<sub>B</sub> = fog of blue density, D<sub>G</sub> = fog of green density, D<sub>R</sub> = fog of red density.)

From Table 4, it is understood that the light-sensitive color printing material according to the present invention is successfully inhibited from formation of fog.

What we claim is:

1. A photographic element comprising a support having thereon one or more layers at least one of which is a light-sensitive silver halide emulsion layer, said element contains a thiosugar having the formula:



wherein R<sub>1</sub> is a hydrogen atom, an alkyl group, or a group of the formula



X is a halogen atom, and Y and Z are individually an alkyl, aryl or aralkyl group; and R<sub>2</sub> is a hydrogen atom or a group of the formula —CH<sub>2</sub>—O—R<sub>3</sub>, and R<sub>3</sub> is an acyl group

said thiosugar being present in an amount effective to inhibit fog.

2. A photographic element as claimed in claim 1 wherein an N-vinyl pyrrolidone polymer is present in said silver halide emulsion layer.

3. A photographic element as claimed in claim 1, wherein said thiosugar is one of the stereoisomers with

respect to the C<sub>(1)</sub> to C<sub>(5)</sub> atoms.

4. A photographic element as claimed in claim 1, wherein said thiosugar is one or two members selected from the group consisting of 1-mercaptop-D-glucose tetraacetate, 1-mercaptop-D-mannose tetraacetate, 1-acetylthio-D-ribose triacetate, 1-acetylthio-D-mannose tetraacetate, butyl tetraacetyl-D-glucose xanthate, tetraacetyl-D-glucose iso-thiuronium bromide, 1-mercaptop-D-xylose triacetate, ethyl triacetyl-D-xylose xanthate and 1-methylthio-D-glucose tetraacetate.

20 5. A photographic element as claimed in claim 1, wherein said N-vinylpyrrolidone polymer is one or two members selected from the group consisting of poly-N-vinyl-2-pyrrolidone, N-vinylpyrrolidone/2-methylimidazolinoacrylic amide copolymer, N-vinylpyrrolidone/acrylic amide copolymer, N-vinylpyrrolidone/2-methylimidazolino-maleamic acid 2-methylimidazole salt copolymer and N-vinylpyrrolidone/morpholinoacrylic amide copolymer.

6. A photographic element as claimed in claim 4, 30 wherein said thiosugar is butyl tetraacetyl-D-glucose xanthate, 1-mercaptop-D-glucose tetraacetate, 1-acetylthio-D-mannose tetraacetate, tetraacetyl-D-glucose iso-thiuronium bromide, 1-acetylthio-D-ribose triacetate or 1-mercaptop-D-mannose tetraacetate and said 35 N-vinylpyrrolidone polymer is poly-N-vinylpyrrolidone.

7. A photographic element as claimed in claim 1, wherein said thiosugar is used in an amount of 10 mg. to 2 g. per mole of silver halide.

40 8. A photographic element as claimed in claim 1, wherein 5-methyl-7-hydroxy-1,3,4-triaza-indene is further incorporated into said silver halide emulsion layer.

9. A photographic element as claimed in claim 1, 45 wherein 1-phenyl-5-mercaptop-tetrazole is further incorporated into said silver halide emulsion.

\* \* \* \* \*